

3,827,886

LIGHT-SENSITIVE SILVER HALIDE  
PHOTOGRAPHIC MATERIALS

Masao Ishihra, Teruhide Haga, Hiroshi Horiuchi,  
Hisashi Yamaguchi and Osakazu Sugino, Tokyo,  
Japan, assignors to Konishiroku Photo Industry  
Co., Ltd., Tokyo, Japan

No Drawing. Continuation of application Ser. No. 52,760,  
July 6, 1970. This application July 3, 1972, Ser. No.  
268,754

Claims priority, application Japan, July 9, 1969,

44/53,767

Int. Cl. G03c 1/06, 1/34, 5/26

U.S. Cl. 96—50 R

3 Claims

## ABSTRACT OF THE DISCLOSURE

A method of preventing fog during rapid development of a light-sensitive silver halide emulsion at elevated temperatures by developing said emulsion in the presence of 4-hydroxy-6-methyl-1,3,3 $\alpha$ ,7-tetrazaindene and at least one of a particular group of quaternary ammonium compounds.

The present invention relates to a light-sensitive silver halide photographic material in which a compound represented by the general formula shown later is used as an antifogging agent in combination with 4-hydroxy-6-methyl-1,3,3 $\alpha$ ,7-tetrazaindene. An object of the present invention is to provide a light-sensitive silver halide photographic material having excellent antifogging properties, particularly one which, even when subjected to quick development treatment, has excellent antifogging properties and has less variation of photographic properties as compared with the case of ordinary development treatment.

Recently, light-sensitive photographic materials have been desired which can be developed quickly by treatment at high temperature in a short period of time. When treated at high temperature, however, light-sensitive photographic materials tend to be increased in fog and are deteriorated in photographic properties, in general.

Light-sensitive photographic materials have heretofore been sensitized by such sensitization methods as sulfur sensitization, reduction sensitization, noble metal sensitization, and sensitization using polyalkylene glycols. Since these methods are liable to degrade the photographic emulsions in antifogging characteristic, in general, there have been used many kinds of antifogging agents. Typical examples of such antifogging agents are 4-hydroxy-6-methyl-1,3,3 $\alpha$ ,7-tetrazaindene and 1-phenyl-5-mercaptopotetrazole. The former compound acts to stabilize the fog of a silver halide photographic emulsion which is under storage and is relatively low in fog-inhibiting effect on a photographic emulsion immediately after its preparation. On the other hand, the latter compound is high in fog-inhibiting effect on a photographic emulsion immediately after its preparation. Ordinarily, therefore, these two compounds are used together to attain the fog-inhibiting effect. However, the 4-hydroxy-6-methyl-1,3,3 $\alpha$ ,7-tetrazaindene is lessened in fog-inhibiting effect during high temperature development, while the 1-phenyl-5-mercaptopotetrazole is strong in desensitizing action, and when it has been incorporated in a photographic emulsion in an amount sufficient to inhibit the fog formation at the time of high temperature development, the photographic emulsion is greatly desensitized and is not practical. Accordingly, in the case of the conventional light-sensitive photographic emulsion containing the said antifogging agents, the degradation of photographic properties during high temperature development is greater than during ordinary development treatment, and it is difficult to expect a sufficient fog-inhibiting effect.

In view of such actual circumstances as mentioned above, we made studies on light-sensitive silver halide photographic emulsions capable of being successfully developed not only by the quick development treatment but also by the ordinary development treatment. As the result, we have found that a light-sensitive silver halide photographic emulsion, which has been incorporated with at least one of the compounds represented by the general formulas (I), (II), (III) and (IV) set forth below in combination with 4-hydroxy-6-methyl-1,3,3 $\alpha$ ,7-tetrazaindene, is markedly lower in degree of desensitization than in the case of the conventional photographic emulsion, shows a high fog-inhibiting effect not only during ordinary development but also at the time of high temperature treatment, and is extremely less in variation of photographic properties.

(I)



(II)



(III)



(IV)



wherein R<sub>1</sub> and R<sub>2</sub> are individually an alkyl or hydroxyalkyl group having 1 to 18 carbon atoms; R<sub>3</sub> is an alkyl or hydroxyalkyl group having 1 to 18 carbon atoms or an aryl or aralkyl group; X is an anion; Z is a non-metal group necessary to form the hetero ring together with the N atom; A is an alkyl, alkenyl, alkynyl, aryl or aralkyl group; and B is  $-(CH_2)_n-$ ,  $-CH_2O(CH_2)_nOCH_2-$ ,



The compounds represented by the above-mentioned general formulas have heretofore been known as sensitizers, as disclosed in U.S. Pat. 2,288,226, and scarcely display fog-inhibiting effects. When used in combination with 4-hydroxy-6-methyl-1,3,3 $\alpha$ ,7-tetrazaindene, however, they show excellent fog-inhibiting effects by virtue of interactions with the said compound, as is clear from the examples set forth later.

Processes for synthesizing the compounds represented by the above-mentioned general formulas have already been reported in many references. For example, the process for synthesizing the compounds from pyridines and alkyl dihalides is disclosed in "Journal of the American Chemical Society," 18, 988 and "Annalen der Chemie," 121, 254; the process for synthesizing quaternary salts from xylene dihalides is disclosed in "Berichte," 34, 2089; the process for synthesizing the compounds from alkylamines or pyridines and alkylhalides is disclosed in "Industrial and Engineering Chemistry," 45, 1022, "Chemical and Engineering News" 30, 1282, and "Journal of the American Chemical Society," 68, 753 and 63, 147; and the process for synthesizing the compounds from azoles and alkylene dihalides or alkyl halides is disclosed in U.S. Pats. 2,425,774 and 2,694,716.

Typical examples of the compounds represented by the aforesaid general formula which are effective for practice of the present invention are as follows:

**4**

30 In adding to a silver halide photographic emulsion, each of the above-mentioned compounds and 4-hydroxy-6-methyl-1,3,3 $\alpha$ ,7-tetrazaindene are brought into the form of, for example, aqueous solutions, alkali solutions or alcohol solutions, either singly or in combination with each other, and are added to the emulsion. The amounts of the 4-hydroxy-6-methyl-1,3,3 $\alpha$ ,7-tetrazaindene and the compound represented by the aforesaid general formula which are to be added to the emulsion are, respectively, 0.05 to 6.0 g. and less than 1 g. per 100 g. of the silver halide. Further, these compounds may be incorporated into any one of the layers constituting a light-sensitive photographic material, such as the protective layer, inter layer, filter layer or other gelatin-containing layer. In this case also, the amounts of the compounds to be incorporated 45 are preferably within the above-mentioned ranges. In any of the above-mentioned cases, the compounds may be added at an optional stage during the steps for production of light-sensitive photographic material.

Light-sensitive silver halide photographic materials 50 obtained in the above manner are quite stable even when subjected to development treatment at a high temperature for a long period of time, and are best suitable for quick development. Further, the photographic materials have excellent photographic properties also in the case 55 where they have been treated under ordinary development conditions. Moreover, they are less affected by the development conditions and have such characteristics that stable photographic properties can always be attained.

The present invention is illustrated in further detail 60 below with reference to examples.

#### Example 1

A gelatino-silver halide photographic emulsion containing 60 g. of silver iodobromide, in which the amount 65 of silver iodide was 1.5 mol percent, was subjected, at the time of second ripening, to gold sensitization. After completion of the ripening, the emulsion was equally divided into 5 portions, and one portion was used as a control while the remaining 4 portions were combined 70 with the compounds shown in Table 1. These emulsions were individually coated on a polyester film base and then dried to prepare samples. The thus prepared samples were treated according to the sensitometry method regulated in JIS-K-7604 and measured in fog and relative speed to obtain the results shown in Table 1.

The compositions of the developers used were as set forth below and the development conditions were as shown in Table 1.

to prepare samples. The thus prepared samples were treated in the same manner as in Example 1 to obtain the results shown in Table 2.

TABLE 2

| Amount<br>added<br>(mg.)  | After development<br>with developer (I)<br>at 40° C. for 30 seconds |                   | After development<br>with developer (II)<br>at 20° C. for 4.5 minutes |                   |
|---------------------------|---------------------------------------------------------------------|-------------------|-----------------------------------------------------------------------|-------------------|
|                           | Fog                                                                 | Relative<br>speed | Fog                                                                   | Relative<br>speed |
| Control                   | 0.28                                                                | 100               | 0.08                                                                  | 81                |
| Compound (A)              | 0.20                                                                | 91                | 0.06                                                                  | 80                |
| Compound (A)              | 0.09                                                                | 51                | 0.06                                                                  | 48                |
| Compound (B)              | 20                                                                  |                   |                                                                       |                   |
| Exemplified Compound (1)  | 0.25                                                                | 90                | 0.09                                                                  | 83                |
| Compound (A)              | 0.09                                                                | 87                | 0.06                                                                  | 80                |
| Exemplified Compound (1)  | 0.09                                                                | 82                | 0.09                                                                  | 83                |
| Exemplified Compound (6)  | 0.20                                                                | 85                | 0.07                                                                  | 81                |
| Compound (A)              | 0.09                                                                | 85                | 0.07                                                                  | 81                |
| Exemplified Compound (6)  | 0.09                                                                | 85                | 0.07                                                                  | 81                |
| Exemplified Compound (17) | 0.23                                                                | 85                | 0.07                                                                  | 81                |
| Compound (A)              | 0.06                                                                | 81                | 0.06                                                                  | 79                |
| Exemplified Compound (17) | 0.06                                                                |                   |                                                                       |                   |

## Developer (I)

|                                | G.   |
|--------------------------------|------|
| Sodium sulfite                 | 70   |
| Hydroquinone                   | 10   |
| Boric anhydride                | 1    |
| Sodium carbonate (monohydrate) | 20   |
| 1-Phenyl-1,3-pyrazolidone      | 0.35 |
| Sodium hydroxide               | 5    |
| 5-Methylbenzotriazole          | 0.05 |
| Potassium bromide              | 5    |
| Glutaraldehyde bisulfite       | 15   |
| Acetic acid                    | 8    |
| Water to make 1 liter.         |      |

## Developer (II)

|                                | G.  |
|--------------------------------|-----|
| Metal                          | 3.5 |
| Anhydrous sodium sulfite       | 60  |
| Hydroquinone                   | 9.0 |
| Sodium carbonate (monohydrate) | 53  |
| Potassium bromide              | 4.0 |
| Water to make 1 liter.         |     |

In the table, the developers (I) and (II) and the compounds (A) and (B) are the same as in Example 1.

From the above table, it is understood that the samples according to the present invention have excellent photographic properties, and that both in the quick development treatment and in the ordinary development treatment, they are free from decrease in sensitivity, show favorable fog-inhibiting effects and are less in variation of photographic properties.

What is claimed is:

1. A method of preventing fog during rapid development at elevated temperatures of a light-sensitive silver halide emulsion in a photographic material which comprises developing said emulsion in the presence of (A) 4-hydroxy-6-methyl-1,3,3 $\alpha$ ,7-tetrazaindene and (B) at least one of the compounds represented by either of the following formulas:



TABLE 1

| Amount<br>added<br>(mg.)  | After development<br>with developer (I)<br>at 40° C. for 30 seconds |                   | After development<br>with developer (II)<br>at 20° C. for 4.5 minutes |                   |
|---------------------------|---------------------------------------------------------------------|-------------------|-----------------------------------------------------------------------|-------------------|
|                           | Fog                                                                 | Relative<br>speed | Fog                                                                   | Relative<br>speed |
| Control                   | 0.31                                                                | 100               | 0.08                                                                  | 82                |
| Compound (A)              | 0.25                                                                | 97                | 0.07                                                                  | 80                |
| Exemplified Compound (21) | 0.21                                                                | 70                | 0.09                                                                  | 83                |
| Compound (A)              | 0.08                                                                | 72                | 0.07                                                                  | 75                |
| Exemplified Compound (21) | 0.08                                                                | 72                | 0.07                                                                  | 75                |
| Compound (A)              | 0.06                                                                | 48                | 0.05                                                                  | 41                |
| Compound (B)              | 0.06                                                                |                   |                                                                       |                   |

In the table, the compound (A) is 4-hydroxy-6-methyl-1,3,3 $\alpha$ ,7-tetrazaindene, and the compound (B) is 1-phenyl-5-mercaptopotetrazole.

From the above table, it is understood that when used singly, the exemplified compound (21) is low in fog-inhibiting effect during high temperature development treatment, but displays quite marked effects when used in combination with the compound (A) and does not suffer from decrease in sensitivity even by the ordinary development treatment, so that the light-sensitive photographic materials of the present invention have excellent photographic properties.

## Example 2

The same emulsion as in Example 1 was equally divided into 9 portions, and one portion was used as a control while the remaining 8 portions were combined with the antifoggants as shown in Table 2. These emulsions were individually coated on a polyester film base and then dried

wherein R<sub>1</sub> and R<sub>2</sub> are individually an alkyl or hydroxyalkyl group having 1 to 18 carbon atoms; R<sub>3</sub> is an alkyl or hydroxyalkyl group having 1 to 18 carbon atoms or a substituted or unsubstituted aryl or aralkyl group; X is an anion; Z is a non-metal group necessary to form a pyridine, quinoline or benzothiazole ring by bonding to the N atom; A is an alkyl, alkenyl, alkynyl, aryl or aralkyl group; and B is  $-(CH_2)_n-$ ,  $-\text{CH}_2\text{O}(\text{CH}_2)_n\text{OCH}_2-$ ,



70  $-\text{CH}_2\text{COCOCH}_2-$  or



75 where n is a positive integer of 1 to 10, and wherein said compounds (A) and (B) are incorporated in said photographic material.

2. A method for developing a light-sensitive silver halide photographic material comprising 4-hydroxy-6-methyl-1,3,3 $\alpha$ ,7-tetrazaindene and at least one of the compounds represented by any of the following general formulas (I), (II), (III) and (IV):



(I)

(II)

(III)

(IV)

—CH<sub>2</sub>—O—CH<sub>2</sub>—, —CH<sub>2</sub>CH<sub>2</sub>—S—CH<sub>2</sub>CH<sub>2</sub>—  
—CH<sub>2</sub>COCOCH<sub>2</sub>— or

—CH<sub>2</sub>OCH<sub>2</sub>CH<sub>2</sub>—S—CH<sub>2</sub>CH<sub>2</sub>OCH<sub>2</sub>—, where *n* is a positive integer of 1 to 10, which comprises developing said material at an elevated temperature.

3. A method as claimed in claim 1 wherein the said compounds are present in at least one of the emulsion layer, interlayer, protective layer and filter layer of said photographic material.

5

10

15

20

25

30

## References Cited

## UNITED STATES PATENTS

|           |        |                |       |         |
|-----------|--------|----------------|-------|---------|
| 2,886,437 | 5/1959 | Piper          | ----- | 96—66 R |
| 2,940,851 | 6/1960 | Beavers et al. | ----- | 96—66.3 |
| 2,944,902 | 7/1960 | Carroll et al. | ----- | 96—107  |
| 3,576,633 | 4/1971 | Henn et al.    | ----- | 96—66.5 |

## FOREIGN PATENTS

|         |        |        |       |         |
|---------|--------|--------|-------|---------|
| 593,411 | 3/1960 | Canada | ----- | 96—66.3 |
|---------|--------|--------|-------|---------|

## OTHER REFERENCES

Accelerated Processing, Photo Methods for Industry, February 1959, pp. 32—35, 72—73, esp. p. 33.

RONALD H. SMITH, Primary Examiner

M. F. KELLEY, Assistant Examiner

## U.S. CL. X.R.

96—48 QP, 95, 109

